

June 10, 1924.

1,496,879

J. H. HIRT

TREATMENT OF ORES

Filed Feb. 2, 1920

Fig. 1,



Fig. 2,



Jules Hector Hirt Inventor  
By his Attorneys  
Penn, Davis, Mann & Elmore

## UNITED STATES PATENT OFFICE.

JULES HECTOR HIRT, OF EL PASO, TEXAS, ASSIGNOR, BY MESNE ASSIGNMENTS, TO MEXICAN NORTHERN MINING AND RAILWAY COMPANY, A CORPORATION OF DELAWARE.

## TREATMENT OF ORES.

Application filed February 2, 1920. Serial No. 355,681.

To all whom it may concern:

Be known that I, JULES HECTOR HIRT, a citizen of the United States, residing at El Paso, in the county of El Paso, State of Texas, have invented certain new and useful Improvements in the Treatment of Ores; and I do hereby declare the following to be a full, clear, and exact description of the invention, such as will enable others skilled in the art to which it appertains to make and use the same.

This invention relates to an improved process of chloridizing ores, concentrates, and other metallurgical products, to convert the metal values into chlorides or oxy-chlorides, which are retained in the ore body and recovered therefrom, for example, by leaching with a suitable solvent. It is a characteristic advantage of the invention that the chloridizing operation is accomplished without objectionable loss of metal values by volatilization.

In the chloridizing of ores, it has been proposed to mix carbonaceous material with the ore and sodium chloride or other chloride, and to bring about the heating of the ore by combustion of the admixed fuel. This method, however, has the objection that overheating is difficult to avoid, owing to the high temperature of ignition and combustion of the fuel; and it is difficult to prevent loss of chlorides by volatilization when the process is carried out in this way. It is also difficult to avoid the presence of excess oxygen and oxidizing conditions during the chloridizing operation.

I have discovered that the objections to such prior proposals can be avoided, and that the ore or other material can be thoroughly chloridized without any objectionable loss of chlorides by volatilization if hot products of fuel combustion, free from excess air, are caused to pass through a body or column of the ore mixed with salt or other chloridizing agent. I have further discovered that a relatively low temperature of heating the ore by this method will suffice for thorough chloridizing, much lower than where the fuel is mixed directly with the ore and burned to supply the heat for the chloridizing. The process of the present invention accordingly avoids the high temperatures resulting from direct

combustion in the ore body or in contact therewith, and effects the chloridizing by means of gaseous products of combustion, free from excess oxygen, which, while still hot, are passed into the ore body admixed with the chloridizing agent. This procedure enables the temperature of the ore column undergoing chloridizing, to be closely regulated, and a much better temperature control secured than is possible where the fuel is mixed directly with the ore and blast roasted.

When the fuel is mixed with the ore, it is difficult to maintain a temperature below about 700° C. since the ignition temperature of the fuel under practical conditions is over 600° C. and the combustion of the fuel in contact with the ore subjects the ore directly to the flame temperature.

According to the present invention, a combustible fuel, such as oil or gas, is burned outside the furnace chamber containing the admixed ore and chloridizing agent, and the products of combustion, free from excess oxygen, are introduced into the charge at a regulated temperature, so that the charge is heated thereby. The regulation of the temperature is thus within the control of the operator. This is of economic importance in the chloridizing of ores for the reason that the metallic chlorides of gold, silver, copper, lead, etc., are volatilized at temperatures much below the ignition temperatures of ordinary fuel combustion. For instance, silver chloride begins to volatilize at about 450° C. gold chloride at about 150° C. etc., and these or somewhat higher temperatures will suffice for the chloridizing operation.

In the presence of combustion products free, or practically free from oxygen, this tendency of the chlorides to volatilize is reduced to a minimum, while it is nevertheless possible to raise the heating temperature to such a point as to effect rapid chloridizing, e. g., to or somewhat above the melting or volatilization temperature of the chloride.

It is a characteristic advantage of the process of the present invention that the ore does not require fine crushing, that it is thoroughly dried before entering the reaction zone even when it contains consider-

able moisture, and that it is subjected to a chloridizing action which insures rapid and thorough chloridizing; while the temperature of the ore column is under the ready control of the operator. Among other advantages of the invention are the high fuel efficiency obtainable, due to the fact that the products of combustion are passed directly through the ore column so that the exit gases are practically cold,—the heat of the gases being used first for effecting the chloridizing and thereafter for preheating the incoming fresh charge.

The present invention, as above noted, is of special value in the chloridizing of copper, lead, silver and gold ores, for the production of the corresponding chlorides without loss thereof by volatilization, even where the chlorides volatilize at relatively low temperatures. As a result of the chloridizing operation, the metal values are converted into chlorides or oxy-chlorides, which are retained in the ore body discharged from the furnace, and subsequently recovered therefrom by leaching.

The ores are preferably oxide or oxidized ore, but sulfide ores may also be treated. The improved process of the present invention can be carried out in different types of apparatus, provided the ore body is subjected to products of combustion which are free from excess oxygen, and which are at a sufficient temperature to insure the chloridizing action, when the ore is subjected to the chloridizing action of a common salt or other chloridizing agent.

A furnace adapted for use in carrying out the method as illustrated in the accompanying drawing in which Figure 1 is a vertical section through the furnace and Figure 2 is the section on the line 2—2 of Figure 1.

A particularly advantageous manner of carrying out the improved process is to feed the ore progressively down through an upright furnace 6 somewhat similar to a lime kiln and to supply the products of combustion to the mixture of ore and chloride near the central part 7 of the furnace. The central part of the furnace may thus be surrounded by a combustion chamber opening into the furnace through a series of openings; or the vertical furnace, if rectangular in section, may have combustion chambers 8 in its side walls and lateral openings 9 therefrom into the furnace chamber containing the charge. Fuel and ore may be introduced through the burners 10. The upright or vertical retort or furnace chamber should preferably have a sufficient height so that the products of combustion will be completely cooled in their upward passage through the incoming charge and so that they will give up their heat to the incoming charge. So also, the reduction in tempera-

ture of the escaping products of combustion assists in preventing any tendency toward escape of the volatile chlorides which are condensed in the cooler portions of the incoming charge and returned to the chloridizing zone. Any excess volatile metal chloride will thus be caused to pass downwardly where it will condense in the cooler portions of the chloridized material prior to its escape from the bottom of the furnace chamber. It will be understood that the furnace or retort will be constructed of suitable material resistant to the chemical action of the materials undergoing reaction therein.

In order to provide for proper cooling of the chloridized material in its passage downwardly through the lower portions of the furnace chamber or retort, such lower portions should be provided with cooling means or should be so exposed that the desired cooling will take place so that the outgoing body of chloridized ore will be discharged at a relatively low temperature, well below that of condensation of any of the volatile chlorides.

With the vertical furnace of the character above referred to, the process can be made continuous by charging the ore together with sodium chloride or other chloridizing agent at the top and regulating the discharge of the cooled chloridized ore at the bottom. The ore itself, both before and after chloridizing, will form an effective seal for the furnace chamber or retort, and the cooler portions of the incoming and outgoing ore bodies will condense any chloride or oxy-chloride vapors that would otherwise tend to escape therefrom.

It is a characteristic feature and advantage of the improved process of the present invention that the body of ore requires maximum heating only at or near the temperature of formation of the chlorides, and that the furnace need be heated for only a portion of its length. That is, the ore body need not be maintained for a prolonged period of time at an elevated temperature in the chloridizing zone.

It is a further advantage of the invention, as above mentioned, that very low temperatures are sufficient therefor, with resulting marked economy in the heat required and reduction of the corrosive action upon the retort or furnace.

If crude oil or fuel is used to supply the products of combustion, such oil may be burned in the combustion chamber with avoidance of excess air and the resulting products of combustion then passed directly into the ore body so that the ore body admixed with the sodium chloride or other chloride, will be subjected to the direct heating action of the products of combustion. While a small amount of excess oxygen may

be tolerated in the process without objectionable volatilization, any considerable excess should be avoided. Higher temperatures, such as those of the flame itself, should 5 likewise be avoided.

The amount of sodium chloride or other chloridizing agent required to be admixed with the ore will vary with the amount of the metal values to be chloridized. It is 10 not necessary to use a large excess of the chloridizing agent, and, for silver, gold and low grade copper ores, as little at 1 or 2%, or even less may suffice, although a larger amount can be used.

15 It is an advantage of the present process that fine grinding of the ore is not necessary, but relatively large lumps of ore can be used provided they are sufficiently porous.

Although the temperature at which 20 sodium chloride will melt and volatilize is a relatively high temperature, nevertheless effective chloridizing can be effected with sodium chloride, according to the process of the present invention, at a much lower 25 temperature, inasmuch as the sodium chloride will react with sulfur dioxide or moisture present in small amount in the products of combustion. For example, where crude oil is used as the fuel for producing the products of combustion, the products of combustion will contain appreciable amounts of steam in a highly reactive form. So also, where the crude oil contains appreciable amounts of sulfur, this will be 30 oxidized and the resulting sulfur dioxide or sulfur trioxide will be present in small amount in the products of combustion and will contribute to the chloridizing process. Where increased amounts of reactive steam 35 or sulfur dioxide are desirable, these can be supplied by adding further amounts of steam in admixture with the products of combustion and by adding small amounts of sulfur, for example, by suspending it in 40 a finely-divided state in the fuel oil.

In a vertical shaft furnace, such as above described, having a furnace chamber adjacent the ore surrounding its central portions for supplying the products of combustion to the shaft at an intermediate point of its height, the effective reacting zone will be at or near the place where the gases are introduced. In the continuous operation of such a furnace, the heated 50 chloridized ore will retain its heat for an appreciable time as it passes downwardly from the chloridizing zone and a further opportunity will thus be permitted in the completion of the chloridizing. The main 55 chloridizing action, however, will take place where the products of combustion enter the shaft or somewhat thereabout inasmuch as the hot gases tend to rise in the shaft and to impart their heat to the incoming charge 60 as it progresses slowly down toward the

main reacting zone. In such a furnace, operated in a continuous manner, the upper portion of the shaft will be a preheating zone for the charge, in which the products of combustion will be cooled, while the lower 70 portion of the shaft will be a cooling zone, in which the hot chloridized ore will be permitted to cool prior to its discharge or withdrawal from the furnace.

Where the ores treated are sulfide ores, 75 containing a small percentage or even a fraction of a percent of metal sulfides, it may be of advantage to introduce a small amount of oxygen with the products of combustion to assist in the oxidation of the 80 sulfur, but, as above pointed out, any such amount of excess oxygen as would give oxidizing conditions and cause appreciable loss by volatilization should be avoided.

Instead of carrying out the process in 85 furnaces constructed as above described, other suitable types of furnaces can be used which will enable the desired heating to be brought about by means of products of combustion in the manner above described. 90

After the ore has been chloridized and the metal values converted into chlorides or oxy-chlorides, the ore is then subjected to a leaching operation for the purpose of extracting therefrom the chlorides or oxy- 95 chlorides so formed. In this leaching operation any suitable solvent can be used which will dissolve the chlorides formed. The ore may thus be leached with a cyanide solvent, with a hyposulfite solution, with a saturated 100 brine (sodium chloride) solution, with an acid brine solution (containing 1 or 2% of hydrochloric or sulfuric acid), a brine solution containing ferric chloride, etc. The ore may thus be leached in any suitable 105 manner which is available for the leaching and extraction of the chloridized values; and the values can be recovered from the leach liquid thus produced in any suitable manner, as will be readily understood. 110

Having thus described my invention, what I claim is:

1. The method of chloridizing ores, metallurgical products and the like, which comprises subjecting a compact body of the same 115 admixed with a suitable chloride to the direct heating action of products of combustion free from any appreciable excess of oxygen; substantially as described.

2. The method of chloridizing ores, metallurgical products and the like, which comprises subjecting the same to the action of a chloridizing agent and to the direct heating action of products of combustion 120 free from any appreciable excess of oxygen, 125 and preventing escape of volatilized chlorides with the escaping products of combustion; substantially as described.

3. The method of chloridizing ores, metallurgical products and the like, which com- 130

5 prises progressing a charge of the ore admixed with a chloridizing agent downwardly through a vertical shaft furnace or retort and heating the same by the introduction of 10 products of combustion free from any appreciable excess of oxygen into the charge at an intermediate point, escape of volatile chlorides with the escaping products of combustion being prevented; substantially as described.

15 4. The method of chloridizing ores, metallurgical products and the like, which comprises progressively feeding a charge of the material to be chloridized through a heating zone, a chloridizing zone, and a cooling zone, and subjecting the material to the action of the chloridizing agent in the chloridizing zone while heating the material by the introduction of hot products of combustion, any objectionable escape of volatile chlorides being prevented; substantially as described.

20 5. The method of chloridizing ores, metallurgical products and the like, which comprises heating a mixture of the material to be chloridized and sodium chloride by introducing hot products of combustion thereto, the products of combustion being substantially free from oxygen and containing 25 constituents reacting with the sodium

chloride to promote the chloridizing action; substantially as described.

6. The method of chloridizing which comprises introducing products of combustion formed externally thereof and free from excess oxygen, to a compact body of ore or like metallurgical material having a chloridizing agent admixed therewith and thereby forming chlorides of the desired metal values. 35

7. The method of chloridizing which comprises introducing products of combustion formed externally thereof, to a compact body of ore or like metallurgical material having a chloridizing agent admixed therewith, thereby forming chlorides of the desired metal values and collecting volatilized chlorides in overlying layers of said material. 40

8. The method of chloridizing which comprises introducing products of combustion formed externally thereof and free from excess oxygen, to a body of ore or like metallurgical material having a chloridizing agent admixed therewith while the body is traveling through a reaction zone and thereby forming chlorides of the desired metal values. 50 55

In testimony whereof I affix my signature.

JULES HECTOR HIRT.